

Aug. 17, 1948.

L. PESSEL

**2,447,362**

## PRODUCTION OF CRYSTALS

Filed Nov. 1, 1945



Fig. 10.

INVENTOR.  
*Leopold Pessel*  
BY 

*ATTORNEY*

## UNITED STATES PATENT OFFICE

2,447,362

## PRODUCTION OF CRYSTALS

Leopold Pessel, Philadelphia, Pa., assignor to  
 Radio Corporation of America, a corporation of  
 Delaware

Application November 1, 1945, Serial No. 626,135

23 Claims. (Cl. 171—327)

1

This invention relates to the art of producing crystals and more specifically to producing synthetically, crystals which exhibit a piezo-electric effect.

One object of this invention is to produce monocrystal bodies, in general, synthetically by recrystallization of finely subdivided crystallizable substances.

Another object is to produce synthetic oscillator plates of quartz or other piezoelectric substances.

Another object is to change the frequency of existing oscillator plates by synthetic crystal growth.

A further object of the invention is to produce synthetic crystals in such a shape and form that a minimum of additional mechanical operations has to be performed to produce a finished oscillator plate.

Another object is to produce a large number of oscillator plates simultaneously, with little frequency deviation between them.

Heretofore the main source of piezoelectric crystals has been naturally occurring crystals of certain minerals, particularly quartz, which were then cut to proper thickness and shape. However, although quartz is a mineral of common occurrence the number of quartz crystals occurring in nature which are suitable for the manufacture of piezoelectric plates is relatively very small. Only those crystals which have a perfect monocrystalline form can be used and the industry has gone to great lengths searching throughout the world for natural quartz deposits having occurring therein crystals of suitable quality. Only a very small percentage of the mined mineral is sent to the laboratories where the crystals are cut and shaped. Yet, such is the uncertainty of prevailing tests which can be used in the field, that of the supposedly perfect crystals finally sent to the laboratory more than half must be discarded when the oscillator plates are being cut.

Another source of piezoelectric crystals has been the well known Rochelle salt or sodium potassium tartrate. Here the prevailing methods have been to grow crystals from the melt or from solution. Rochelle salt crystals, however, have proven unsuitable for use at high frequencies and have mechanical limitations such as softness and high solubility.

Certain methods similar to those used in making Rochelle salt crystals have been tried in making suitable quartz crystals but the results have been disappointing since the product is inferior in both size and quality to the crystals which occur naturally.

2

The present invention represents a distinct change from any of the above described methods and can be applied not only to quartz but to tourmaline, Rochelle salt, and, in fact, to the formation of any crystalline material.

In general, the finely subdivided substance, for example, powdered quartz or silica, is mixed with a small proportion of a solvent. A crystallization catalyst may be added, if speed of reaction is desired. In the case of quartz this catalyst may be a substance which gives an alkaline reaction such as the hydroxides of the alkali and alkaline earth metals as well as some of the stronger organic bases. Other types of catalyst which have been found useful are the inorganic fluoride salts and hydrofluoric acid. Although these catalysts are preferred in the case of quartz the invention contemplates the use, in general, of any substance which catalyzes the crystallization of the substance the crystal of which is being formed. The mixture is compressed into a substantially plate-shaped body and maintained at elevated pressure and preferably at elevated temperature. The compressed body is subjected to high-frequency oscillations by means of suitably spaced electrodes. One frequency component is preferably the natural mechanical vibration frequency of the compressed body. A supersonic frequency component may be added. It is also possible to use other high frequencies of alternation which will produce the desired vibrations in the compressed body.

The invention described herein is based upon recrystallization of finely divided microcrystalline material or the crystallization of finely divided amorphous material. Novel features are shown for causing such crystallization to take place and to proceed in such an oriented manner that the ultimate result is a body showing the characteristics of a monocrystal.

The invention will now be described more specifically as it relates to quartz bearing in mind, however, that the same general principles apply in the case of other substances.

It is well known that quartz or silica is very slightly soluble in water. This solubility increases when the material is powdered and this increase depends upon the degree of subdivision of the particles. In addition, the solubility is increased by raising the temperature and pressure. Further increases in solubility are caused by the presence of other substances. Some of those substances which have been found particularly useful in practicing the invention are the alkalies in which the metal is of the class of alkali or

alkaline earth metals, as well as strong organic bases. Other classes of substances found useful are the fluoride salts and hydrofluoric acid.

The material used should be extremely subdivided silica, such as powdered quartz, chalcedony, hydrated silica, or amorphous silica. The particles are preferably of 10 micron diameter or smaller, although coarser particles may be present.

The powdered silica is mixed with a small amount of water which amount is not fixed but depends upon particle size and shape as well as upon other operating conditions. To this mixture is preferably added a small amount of one of the catalysts heretofore enumerated in order that recrystallization may be accelerated. The quantity of catalyst may vary between a mere trace and an amount corresponding to its saturation limit in the water present. If it is not desired to speed up the crystallization process the catalyst may be omitted.

The prepared mixture is then treated by the method presently to be described using suitable apparatus which is diagrammatically represented in the various figures, of which:

Fig. 1 represents diagrammatically a longitudinal section view of apparatus suitable for applying a single high frequency component.

Fig. 2 represents a modification in which an additional supersonic component is added at right angles to the high frequency component.

Fig. 3 represents a modification in which the high frequency electrodes are placed at an angle to the plane of the faces of the chamber.

Fig. 4 represents a modification in which the high frequency electrodes are placed parallel to the main faces of the oscillator plate but having the electrodes of the supersonic component at some angle other than a right angle in relation to the high frequency electrodes.

Fig. 5 shows a modification in which the centers of the high frequency electrodes are laterally displaced.

Fig. 6 shows a variation of the above in which the electrodes of the supersonic component are also at an angle other than a right angle to the planes of the high frequency electrodes.

Fig. 7 shows a modification in which quartz oscillator plates are used in place of metal electrodes.

Fig. 8 represents a modification by means of which a quartz crystal of given frequency may be changed into a thicker crystal of lower frequency.

Fig. 9 represents a modification in which more than two electrodes are used and in which the fields are parallel.

Fig. 10 represents a modification in which more than two electrodes are used and in which the fields are not parallel.

Fig. 11 represents a view of the apparatus shown diagrammatically in Fig. 1 but taken at right angles to the view shown in Fig. 1.

The finely powdered silica 22 with the water and catalyst added is packed in the compartment as shown in Fig. 1. The mass is raised to an elevated temperature which may be anywhere from slightly above room temperature, as 50° C. up to the inversion temperature of quartz (573° C.). A preferred temperature is the critical point of water (374° C.). The temperature is controlled by resistance heaters 14 connected to the A. C. mains by conductors 20. Any suitable A. C. current controlling means of conventional

design may be used for raising or lowering the current. In this figure, 11 represents the remaining sides of the chamber which may be constructed of insulating material such as glass or other ceramic substance. Any rigid insulator which will not be affected by the temperature and pressure used may be made use of.

Where it is not necessary or desirable to speed up the solution process, ordinary room temperature may be used. As in the case of the catalyst, increased temperature is used only to speed up the process and may be omitted if desired.

Elevated pressure is then applied to top plate 1 through shaft 15 in order to compact the particles and accelerate the recrystallization reaction. This pressure is preferably not less than the vapor pressure of water at the temperature selected but may be considerably higher.

An electric field alternating at high frequency is maintained between electrodes 1 and 2 which are insulated from each other. This high frequency field may be supplied by any conventional type of high frequency oscillator such as shown diagrammatically at A. The electrodes are connected to the generator through conductors 19.

Where only a single alternating field component is used it is preferable that said frequency correspond to the natural vibration frequency of the crystal being formed. However, some other frequency suitable for setting up the necessary mechanical strains may be used. For quartz this frequency may vary all the way from 50 kilocycles per second (50,000 cycles/second) to 10 megacycles per second (10,000,000 cycles/second) and even higher.

The frequency with which a quartz plate oscillates is represented by the equation

$$f = \frac{K}{t}$$

where  $f$  = the fundamental thickness-mode in megacycles/second,  $t$  is thickness in mils of an inch and  $K$  is a constant, 99 for the V2 cut quartz crystal and 66 for the V1 cut (see U. S. patent to Gerber, 2,304,760). Since the frequency is inversely proportional to the thickness, the greater the thickness the lower will be the frequency of the oscillator plate produced. The frequency range mentioned represents about the practical limits of commercially usable quartz oscillator plates at the present time although it is possible to get some results with both higher and lower frequencies.

Although not wishing to be limited to the theory of what supposedly occurs during the above-described process it is thought to take place as follows:

When the mixture of finely divided silica, water and catalyst is subjected to elevated temperature and pressure, some of the silica goes into solution. Since this reaction takes place in a closed system some of the silica first dissolves then redeposits in accordance with the principles of phase equilibrium resulting in a gradual growth of the crystalline particles. This growth should theoretically proceed until the whole mass has been transformed into one single crystal. However, when no means are provided for orienting the crystallites, growth takes place in a haphazard manner as to crystal orientation. In addition, as the crystallites grow there is a corresponding decrease in the active reaction area. The result of these two factors, if allowed to proceed without the conditions prescribed by the present invention, would be the formation

of a crystalline aggregate showing extensive twinning rather than formation of a monocrystal.

When the microcrystalline or amorphous powder is compressed, as in the present invention, to such an extent that it behaves like a rigid body, the possibility is given to direct the orientation of the growing particles into uniform axial directions. It is well known that crystal growth shows directional response to mechanical stresses. In the method described, such mechanical stresses are created by subjecting the compressed mixture to one or more alternating electric fields.

There are various modifications of the method which may be used to advantage some of which may be utilized to produce crystals of special types.

In the modification shown in Fig. 2, there is used in addition to the high frequency field, a source of supersonic vibrations B connected through conductors 21 to end electrodes 16. The use of these supersonic vibrations aids in the mechanical reorientation of the particles and thus promotes oriented crystallization. The frequency range useful here is 15-50 kilocycles/second.

In order to produce quartz oscillator plates of other than the X-cut type other modifications of the method may be used. As in Fig. 3, the high frequency field may be applied by electrodes 26, 27 whose surfaces are placed at some angle with respect to the main faces of the insulating plates 12 and 25.

In Fig. 4 the high frequency electrodes 1 and 2 are placed as in Fig. 1 but the electrodes 17 connected to the source B of supersonic vibrations are placed at an angle to the high frequency electrodes.

In order to provide for a high frequency field which will travel at an angle through the powdered mass, the electrodes may be arranged as at 3 and 4 in Fig. 5. Here the high frequency electrodes are set in the insulating plates 13 with their centers laterally displaced.

A further modification is shown in Fig. 6 in which the electrodes connected to the source of supersonic vibrations are also set at an angle to the main faces of the oscillating plate being formed.

It has also been found desirable to sometimes set up two or more high frequency fields in orienting the crystallites. Such an arrangement is shown in Fig. 9 in which the fields are parallel. Electrodes 7 and 8, when connected to high-frequency source A<sub>2</sub> produce one field while electrodes 9 and 10 connected to high frequency source A<sub>1</sub>, produce another field parallel to the first. The fields may have the same or different frequencies.

In Fig. 10 the electrodes 9' and 10' produce a field which is not parallel to that set up between electrodes 7' and 8'.

The alternating mechanical stresses required for oriented recrystallization are best produced, in piezoelectric substances, by an alternating electric field. In other materials, however, such stresses may be applied to the parent body by an oscillating element or elements, such as quartz oscillator plates vibrating at the proper frequencies which may, wholly or partly, replace the metal electrodes previously described. This is illustrated in Fig. 7 where 5 and 6 are hooked up to high frequency oscillator C. Electrodes 27 and 28 are metal plates through which quartz plate 5 is caused to vibrate. Electrodes 29 and

30 perform a similar function for quartz plate 6.

The invention may also be used in building up the dimensions of existing quartz oscillator plates. As illustrated in Fig. 8, a quartz oscillator plate 23 is packed in a powdered silica, water, catalyst mixture 22. Either a high frequency field only may be applied or a two component field of both high frequency and supersonic vibrations may be used. In this way the original crystal may be made larger.

The invention has been described mainly in connection with the manufacture of synthetic quartz crystals. However the method may be applied to the production of other crystalline materials so long as the fundamental conditions are met.

These conditions are:

1. The material is placed in a very fine state of subdivision.

20 2. A liquid is added in which the finely divided material is but slightly or moderately soluble.

3. A crystallization catalyst is desirable although not absolutely necessary.

25 4. Elevated temperature is used when accelerated reaction is desired.

5. Elevated pressure of sufficient degree is used to compress the mixture so that it acts as a rigid body.

30 6. An alternating field of one or more components is used, at least one of which is preferably the natural mechanical vibration frequency of the parent body.

While in some cases it is desired to produce a crystal which has most of the same properties as one occurring naturally, it is possible to produce crystals which are distinctly different. For example, the synthetic crystals may have different lattice constants than those of natural origin. This is possible because of the fact that the synthetic crystals have been produced under mechanical strains not present in the environment when the natural crystals were formed.

In the illustrations the top plate of the compartment is assumed to be movable to provide for exerting pressure on the mass and in all cases means are assumed for suitably heating the assembly where this is desired.

The method of heating the assembly is not by any means limited to the use of resistance wire heating elements. For example, the metal electrodes may be heated by induction and the heat thus transferred to the powdered mass. Also it is feasible to use high frequency dielectric heating in which case the heat is induced directly within the powdered substance.

I claim as my invention:

1. The process of producing a substantially monocrystalline body comprising mixing a powder of a crystallizable substance with a liquid 50 capable of bringing about partial solution of said substance, compressing said mixture within a compartment, subjecting the compressed mixture to elevated temperature, and subjecting the compressed, heated mixture to high-frequency vibrations until substantially all of the mixture has crystallized into a solid body.

2. The process of producing a substantially monocrystalline body comprising mixing a powder of a crystallizable substance with a liquid 70 capable of bringing about partial solution of said substance to which a catalyst of crystallization is added, compressing said mixture within a compartment, subjecting the compressed mixture to elevated temperature, and subjecting the compressed, heated mixture to high-frequency vibra-

tions until substantially all of the mixture has crystallized into a solid body.

3. The process of producing a substantially monocrystalline body comprising mixing a powder of a crystallizable substance with a liquid capable of bringing about partial solution of said substance, compressing said mixture within a compartment, and subjecting the compressed mixture to high-frequency vibrations until substantially all of the mixture has crystallized into a solid body.

4. The invention as set forth in claim 1, characterized by the high-frequency vibrations being applied through the medium of insulated metal electrodes.

5. The invention as set forth in claim 1, characterized by the high-frequency vibrations being applied through the medium of piezoelectric oscillator plates.

6. The invention as set forth in claim 1, characterized by said mixture being compressed into a substantially plate-shaped body and said high-frequency vibrations being set up by an alternating electric field of a frequency corresponding to the natural mechanical vibration frequency of said body.

7. The invention as set forth in claim 1, characterized by said mixture being compressed into a substantially plate-shaped body and said high-frequency vibrations being set up by an alternating electric field one frequency component of which is the natural mechanical vibration frequency of the compressed body and another frequency component of which is in the supersonic range.

8. The invention as set forth in claim 1, characterized by the mixture being compressed into a substantially plate-shaped body, said high-frequency vibrations being set up by an alternating electric field which is not vertical to the main plate faces of said body.

9. The invention as set forth in claim 1, characterized by the mixture being compressed into a substantially plate-shaped body, said body being subjected to alternating electric fields, the fields being in a direction not parallel to each other, one field alternating at the natural mechanical vibration frequency of said body and another field alternating at a frequency in the supersonic range.

10. The invention as set forth in claim 1, characterized by the crystallizable substance being capable of forming piezoelectric crystals.

11. The process of producing a quartz oscillator plate comprising mixing finely divided silica with water, compressing the mixture into a substantially plate-shaped body within a compartment, heating the mixture to a temperature between 50° C. and 573° C. while maintaining a pressure not lower than the vapor pressure of water at said temperature, and maintaining an alternating electric field across the body.

12. The process of claim 11, characterized by the water containing a dissolved crystallization catalyst.

13. The process of claim 11, characterized by the water containing a dissolved crystallization catalyst, said catalyst being a compound which is alkaline in nature.

14. The process of claim 11, characterized by the water containing a dissolved crystallization catalyst, said catalyst being a compound selected from the group consisting of hydrofluoric acid and metallic fluorides.

15. The process as set forth in claim 11, characterized by the alternating electric field being of a frequency corresponding to the natural mechanical vibration frequency of the compressed body.

16. The process as set forth in claim 11, characterized by said alternating electric field having more than one component, one of which is the natural mechanical vibration frequency of the compressed body and another component of which is a frequency in the supersonic range.

17. The process as set forth in claim 11, characterized by more than one type of alternating field being maintained across the compressed body, the direction of which fields is not parallel to each other, and at least one of said directions being not vertical to the main faces of the plate, the frequency of one field being the natural mechanical vibration frequency of the compressed body, the frequency of another field being in the supersonic range.

18. The process of superimposing oriented growth upon a monocrystal body comprising packing around said body a mixture consisting of the finely subdivided substance of said body and a solvent in which said substance is slightly soluble, exposing said combination of body and mixture to elevated temperature and pressure and maintaining across said combination an alternating electric field.

19. The invention as set forth in claim 18, characterized by the body being a quartz plate oscillator.

20. The process as set forth in claim 18, characterized by the alternating electric field being of a frequency corresponding to the natural vibration frequency of the compressed combination.

21. The invention as set forth in claim 18, characterized by said alternating field having more than one component, one of which is of a frequency corresponding to the natural mechanical vibration frequency of said combination and another of which is a frequency in the supersonic range.

22. A monocrystalline body produced by oriented growth of finely divided crystallizable substance in the presence of a solvent for said substance under the influence of elevated temperature, pressure, and an alternating electric field.

23. A monocrystalline body produced by oriented growth of finely divided silica in the presence of a small amount of a solvent for said substance under the influence of elevated temperature, pressure and an alternating electric field.

LEOPOLD PESSEL.

#### REFERENCES CITED

65 The following references are of record in the file of this patent:

#### UNITED STATES PATENTS

|           |          |              |
|-----------|----------|--------------|
| Number    | Name     | Date         |
| 1,886,234 | Meissner | Nov. 1, 1932 |